

## 1

3,309,242

 HIGH-CARBON PRECIPITATION-HARDENING  
AUSTENITIC STEEL ALLOY

Horace Pops, Wilkinsburg Borough, Pa., assignor to  
United States Steel Corporation, a corporation of Dela-  
ware  
No Drawing. Filed Oct. 1, 1964, Ser. No. 400,907  
4 Claims. (Cl. 148—38)

This invention relates to high-carbon precipitation-harden-  
ing austenitic iron alloys characterized by high tem-  
perature tensile strength suitable for aircraft and missile  
uses.

Aircraft and missile structures require alloys that will  
retain strength in the range of 1000 to 1500 F. Presently used materials generally are low-carbon, chromium,  
nickel, iron alloys containing titanium as a major harden-  
ing agent together with molybdenum, vanadium and alu-  
minum. Strengthening of these alloys is accomplished by  
precipitation or age-hardening and is usually attributed to  
internal lattice strains produced by the precipitation of  
intermetallic compounds such as Ni<sub>3</sub>(TiAl). At high  
temperatures the precipitates agglomerate to larger par-  
ticles and thus lose their effectiveness. The carbon con-  
tent of titanium-bearing high-temperature alloys is kept  
at a minimum since with increased carbon contents, the  
titanium acts as a carbide stabilizer and forms relatively  
stable titanium carbide dispersoids so that the matrix is  
depleted of titanium and is therefore not available as a  
precipitation-hardening element. High-carbon, high-tem-  
perature iron alloys are also known; these are usually  
strengthened by the precipitation of chromium carbides  
and are used mainly for valves and the like. However  
such steels have inferior mechanical properties at the  
higher temperatures associated with aircraft and missile  
applications.

It is an object of this invention to provide an austenitic  
iron alloy having a considerably higher level of strength

## 2

for high temperature service because the zirconium carbide  
particles, which form, become agglomerated and  
segregate in the as-cast ingots. On the other hand, I have  
discovered that with relatively high amounts of carbon  
and zirconium, a large number of uniformly dispersed  
zirconium carbide dispersoids are formed and conse-  
quently no internal stress raisers are produced because  
of the uniform distribution. In addition to this disper-  
sion strengthening mechanism, one or more phases pre-  
cipitate out of the matrix during aging heat treatments  
thereby extending the high strength characteristic of the  
steel over longer periods at elevated temperature. Thus  
the mechanical properties of the alloy of this invention are  
believed to be obtained by a superimposition of multiple  
strengthening mechanisms. Moreover despite the large  
volume fraction of carbide particles, the alloy of this  
invention can be readily hot or cold swaged or machined.

The austenitic iron alloy of my invention has the fol-  
lowing compositional range by weight percent:

|    |            |       |            |
|----|------------|-------|------------|
| 20 | Carbon     | ----- | .51 to .60 |
|    | Chromium   | ----- | 10 to 20   |
|    | Nickel     | ----- | 15 to 25   |
|    | Zirconium  | ----- | 2.0 to 4.0 |
|    | Titanium   | ----- | 2.0 to 4.0 |
| 25 | Molybdenum | ----- | 2.0 to 4.0 |
|    | Tungsten   | ----- | 2.0 to 4.0 |
|    | Cobalt     | ----- | 2.0 to 4.0 |
|    | Boron      | ----- | Up to .008 |

30 balance substantially iron and incidental residuals or im-  
purities. In the latter regard, residuals and impurities  
include not only the normal small amounts of phospho-  
rus, sulphur and dissolved gases present in steels but also  
manganese, silicon and aluminum commonly present as  
35 the results of manufacturing processes; the latter elements  
being unnecessary to the properties of the present alloy  
but not deleterious thereto in amounts up to 1.0% each.

The following heats of steel will illustrate the invention:

TABLE I

| Steel  | Zr   | Ti   | C    | Mo   | W    | B      | Co   | Cr | Ni | Fe   |
|--------|------|------|------|------|------|--------|------|----|----|------|
| 1----- | 2    | 4    | 0.8  | 2    | 2    | 0.008  | 4    | 15 | 20 | Bal. |
| 2----- | 2.88 | 2.81 | 0.68 | 2.92 | 3.1  | 0.0042 | 2.98 | 15 | 20 | Bal. |
| 3----- | 2.98 | 3.30 | 0.57 | 2.95 | 3.11 | 0.004  | 2.92 | 15 | 20 | Bal. |
| 4----- | 2.99 | 3.3  | 0.56 | 2.93 | 2.98 | 0.000  | 2.96 | 15 | 20 | Bal. |

and improved ductility at temperatures above about 1200°  
F. than available heretofore.

A further object of this invention is to provide a steel  
having a matrix that is strengthenable by dispersion of  
relatively stable carbide particles as well as by precipita-  
tion hardening.

I have discovered that the foregoing objects can be ob-  
tained in an austenitic chromium nickel steel containing  
high carbon within a restricted range together with limited  
amounts of zirconium, titanium, molybdenum, tungsten  
and cobalt; further that the inclusion of a small amount  
of boron in the composition is very beneficial. Small  
additions of zirconium are not customary in iron alloys

55 The tensile strength at various test temperatures of  
the foregoing steels after precipitation hardening is listed  
in the following Table II along with that of A-286 steel  
which is sometimes used for high temperature service.  
A-286 is a commercially available steel of the low car-  
bon, chromium, nickel, titanium and iron type. As ap-  
parent upon comparison of the properties of steels 4 and  
A-286, the present invention affords materials of con-  
siderably higher strength at elevated temperature than  
available heretofore. The ultimate strength of steel 4 is  
65 about 55% greater at 1500° F. than that of A-286 while  
its yield strength at this temperature is about 160%  
greater. Moreover steel 3 which is essentially the same

as steel 4, except for the presence of 0.004% boron affords an even more remarkable result showing improvements in both tensile and yield strengths of better than 45% at 1300° F. and of more than 100% at 1500° F. As is indicated by comparing the elongations of steels 3 and 4, boron markedly increases the elevated temperature strength of the alloys without lowering the ductility. The effects of boron however are lost when the carbon content of the alloys is increased, see steel 1. That the carbon content must be closely controlled is further evident from steels 2 and 3, wherein a relatively small increase from .57 to .68% has resulted in a large drop in the tensile strength.

TABLE II.—TENSILE AND YIELD STRENGTHS AND ELONGATION FOR STEELS 1, 2, 3, 4 AND A-286 AT TEMPERATURES INDICATED

| Steel              | Test Temperature (°F.) | Tensile Strength (p.s.i.) | Yield Strength .02% Offset (p.s.i.) | Average Elongation in 1", Percent |
|--------------------|------------------------|---------------------------|-------------------------------------|-----------------------------------|
| 1 <sup>1</sup>     | 68                     | 143,700                   | 92,000                              | 10.3                              |
|                    | 1,000                  | 113,300                   | 84,600                              | 11.0                              |
|                    | 1,300                  | 104,400                   | 91,600                              | 9.6                               |
|                    | 1,500                  | 47,000                    | 44,400                              | 15.7                              |
|                    | 1,650                  | 17,500                    | 16,800                              | 36.5                              |
| 2 <sup>1</sup>     | 68                     | 140,000                   | 111,100                             | 13.4                              |
|                    | 1,000                  | 114,800                   | 90,100                              | 9.2                               |
|                    | 1,300                  | 108,100                   | 84,300                              | 11.5                              |
|                    | 1,500                  | 37,300                    | 35,100                              | 18.1                              |
|                    | 1,650                  | 21,000                    | 20,100                              | 42.0                              |
| 3 <sup>1</sup>     | 68                     | 153,000                   | 128,300                             | 6.0                               |
|                    | 1,100                  | 160,900                   | 124,000                             | 7.2                               |
|                    | 1,300                  | 131,300                   | 109,700                             | 9.4                               |
|                    | 1,500                  | 65,600                    | 57,600                              | 28.0                              |
|                    | 1,650                  | 21,500                    | 19,000                              | 34.5                              |
| 4 <sup>1</sup>     | 68                     | 146,000                   | 98,000                              | 7.8                               |
|                    | 1,000                  | 125,500                   | 101,400                             | 9.2                               |
|                    | 1,300                  | 107,200                   | 81,300                              | 13.6                              |
|                    | 1,500                  | 48,100                    | 43,700                              | 25.2                              |
|                    | 1,650                  | 20,200                    | 18,900                              | 30.6                              |
| A-286 <sup>2</sup> | 68                     | 152,000                   | 98,000                              | 20.0                              |
|                    | 1,000                  | 130,000                   | 87,000                              | 16.0                              |
|                    | 1,100                  | 121,000                   | 85,000                              | 13.0                              |
|                    | 1,300                  | 88,000                    | 75,000                              | 4.0                               |
|                    | 1,500                  | 31,000                    | 17,000                              | 14.0                              |
|                    | 1,650                  | 18,000                    | —                                   | 52.0                              |

<sup>1</sup> 1/2 hr. at 1,850° F. + 10 hrs. 1,300° F.

<sup>2</sup> 1/2 hr. at 1,800° F. + 13 hrs. 1,325° F.

TABLE III.—EFFECT OF AGING TIME UPON HIGH TEMPERATURE TENSILE STRENGTH AT 1,300° F. FOR STEEL 3

| 5  | Solution Treatment |             | Aging Treatment |             | Tensile Strength (p.s.i.) | Yield Strength .02% Offset (p.s.i.) | Average Elong. in 1", percent |
|----|--------------------|-------------|-----------------|-------------|---------------------------|-------------------------------------|-------------------------------|
|    | Temp. (° F.)       | Time (hrs.) | Temp. (° F.)    | Time (hrs.) |                           |                                     |                               |
| 10 | 1,850              | 1/2         | 1,300           | 1           | 120,300                   | 93,800                              | 10.8                          |
|    | 1,850              | 1/2         | 1,300           | 10          | 131,300                   | 109,700                             | 9.4                           |
|    | 1,850              | 1/2         | 1,300           | 100         | 133,900                   | 106,500                             | 14.7                          |
|    | 1,850              | 1/2         | 1,300           | 400         | 118,800                   | 95,600                              | 12.1                          |
|    | 1,850              | 1/2         | 1,300           | 750         | 114,200                   | 92,300                              | 13.6                          |
|    | 2,000              | 1/2         | 1,300           | 1,000       | 113,200                   | 86,900                              | 14.2                          |
|    | 2,000              | 1/2         | 1,300           | 10          | 124,700                   | 113,800                             | 9.6                           |
|    | 2,000              | 1/2         | 1,300           | 100         | 127,800                   | 113,500                             | 12.7                          |
|    | 2,000              | 1/2         | 1,300           | 400         | 93,600                    | 80,600                              | 15.9                          |
|    | 2,000              | 1/2         | 1,300           | 750         | 108,100                   | 87,600                              | 22.4                          |
| 15 | 2,000              | 1/2         | 1,300           | 1,000       | 91,200                    | 75,100                              | 14.9                          |
|    | 2,150              | 1/2         | 1,300           | 0           | 92,500                    | 52,100                              | 22.3                          |
|    | 2,150              | 1/2         | 1,300           | 1           | 89,600                    | 53,800                              | 12.1                          |
|    | 2,150              | 1/2         | 1,300           | 10          | 108,100                   | 83,300                              | 11.7                          |
|    | 2,150              | 1/2         | 1,300           | 100         | 117,900                   | 93,100                              | 13.9                          |
|    | 2,150              | 1/2         | 1,300           | 400         | 118,100                   | 101,000                             | 15.0                          |
|    | 2,150              | 1/2         | 1,300           | 750         | 113,300                   | 92,300                              | 28.5                          |
|    | 2,150              | 1/2         | 1,300           | 1,000       | 94,800                    | 81,100                              | 13.2                          |
|    | 20                 | —           | —               | —           | —                         | —                                   | —                             |

TABLE IV.—EFFECT OF AGING TEMPERATURE UPON HIGH TEMPERATURE TENSILE STRENGTH AT 1,300° F. FOR STEEL 3

| 30 | Solution Treatment |             | Aging Treatment |             | Tensile Strength (p.s.i.) | Yield Strength .02% Offset (p.s.i.) | Average Elong. in 1", percent |
|----|--------------------|-------------|-----------------|-------------|---------------------------|-------------------------------------|-------------------------------|
|    | Temp. (° F.)       | Time (hrs.) | Temp. (° F.)    | Time (hrs.) |                           |                                     |                               |
| 35 | 1,850              | 1/2         | 1,200           | 10          | 122,700                   | 94,000                              | 15.9                          |
|    | 1,850              | 1/2         | 1,300           | 10          | 131,300                   | 109,700                             | 9.4                           |
|    | 1,850              | 1/2         | 1,400           | 10          | 124,500                   | 98,700                              | 7.0                           |
|    | 1,850              | 1/2         | 1,500           | 10          | 95,000                    | 69,400                              | 14.5                          |
|    | 1,850              | 1/2         | 1,600           | 10          | 94,200                    | 59,000                              | 22.1                          |
|    | 2,000              | 1/2         | 1,200           | 10          | 90,600                    | 66,000                              | 15.5                          |
|    | 2,000              | 1/2         | 1,300           | 10          | 124,700                   | 113,800                             | 9.6                           |
|    | 2,000              | 1/2         | 1,400           | 10          | 93,700                    | 80,300                              | 9.1                           |
|    | 2,000              | 1/2         | 1,500           | 10          | 71,700                    | 54,400                              | 17.6                          |
|    | 2,000              | 1/2         | 1,600           | 10          | 71,400                    | 43,900                              | 19.1                          |
| 40 | 2,150              | 1/2         | 1,200           | 10          | 99,500                    | 66,300                              | 23                            |
|    | 2,150              | 1/2         | 1,300           | 10          | 106,100                   | 83,300                              | 11.7                          |
|    | 2,150              | 1/2         | 1,400           | 10          | 111,800                   | 87,100                              | 6.8                           |
|    | 2,150              | 1/2         | 1,500           | 10          | 90,500                    | 61,700                              | 11.8                          |
|    | 2,150              | 1/2         | 1,600           | 10          | 98,500                    | 60,400                              | 22.4                          |
|    | 2,150              | 1/2         | —               | —           | —                         | —                                   | —                             |
|    | 2,150              | 1/2         | —               | —           | —                         | —                                   | —                             |
|    | 2,150              | 1/2         | —               | —           | —                         | —                                   | —                             |
|    | 2,150              | 1/2         | —               | —           | —                         | —                                   | —                             |
|    | 2,150              | 1/2         | —               | —           | —                         | —                                   | —                             |

In general and as evident from Table III, solution annealing at temperatures toward the lower end of the range 50 1800 to 2200° F. will produce somewhat higher levels of strength. Annealing time is preferably held to the minimum needed to achieve substantially uniform temperature throughout the alloy. While this will vary with thickness of section, a half hour at temperature is in most instances sufficient.

As also evident from Table III, considerably longer times are involved in the precipitation treatment; aging for 60 100 hours or more at 1300° F. being required to develop maximum strength. However it will be noted that the increase in strength with times longer than 10 hours is minor; consequently treatment for longer than about 10 hours are uneconomical and may even be detrimental.

The effect of aging temperature at a constant treating time of 10 hours is illustrated in Table IV. It will be noted 65 that the optimum aging temperature rises to about 1400° F. as the temperature used in the solution anneal is increased. More important however is the fact that the highest strength level is achieved by solution annealing at about 1850° F., in combination with aging at about 70 1300° F. It is apparent that lower aging temperatures, e.g. 1200° F., are usable but would require extension of the time of treatment, while higher aging temperature, e.g. 1500° F. should be avoided since the strength level drops even when the treating time is drastically shortened. The latter is illustrated by the data of Table V.

The composition of the A-286 steel included in the foregoing table had the following composition:

|    |       |
|----|-------|
| C  | 0.045 |
| Mn | 1.35  |
| Si | .95   |
| P  | .02   |
| S  | .02   |
| Cr | 15.5  |
| Ni | 26.0  |
| Mo | 1.25  |
| Ti | 1.95  |
| V  | .3    |
| Al | .20   |

The properties of the alloys of the present invention are developed by heating treatment involving a solution anneal at temperature ranging from about 1800 to 2200° F. followed by a precipitation or aging treatment at a lower temperature.

The effects of variations in treating conditions are illustrated by the data of Tables III, IV and V. While the tabulated data are specific to steel 3 when tested at 1300° F., they may be considered typical of all the compositions of the present invention as regards the variation in properties to be expected with variations in temperature of solution anneal and the time and temperature used in the precipitation treatment.

TABLE V.—EFFECT OF TIME AND TEMPERATURE OF AGING ON MECHANICAL PROPERTIES OF STEEL 3 AS DETERMINED BY TENSILE TESTS AT 1,800° F.

| Solution Treatment |             | Aging Treatment |             | Tensile Strength (p.s.i.) | Yield Strength (p.s.i.) | Average Elong. in 1", percent | 5 |
|--------------------|-------------|-----------------|-------------|---------------------------|-------------------------|-------------------------------|---|
| Temp. (° F.)       | Time (hrs.) | Temp. (° F.)    | Time (hrs.) |                           |                         |                               |   |
| 1,850              | 1/2         | 1,300           | 1           | 120,300                   | 93,800                  | 10.8                          |   |
| 1,850              | 1/2         | 1,300           | 10          | 131,300                   | 109,700                 | 9.4                           |   |
| 1,850              | 1/2         | 1,500           | 1           | 103,700                   | 87,500                  | 19.8                          |   |
| 1,850              | 1/2         | 1,500           | 10          | 95,000                    | 69,400                  | 14.5                          |   |
| 2,150              | 1/2         | 1,300           | 1           | 89,600                    | 53,800                  | 12.1                          |   |
| 2,150              | 1/2         | 1,300           | 10          | 106,100                   | 83,300                  | 11.7                          |   |
| 2,150              | 1/2         | 1,500           | 1           | 100,100                   | 87,600                  | 14.8                          |   |
| 2,150              | 1/2         | 1,500           | 10          | 90,500                    | 61,700                  | 11.8                          |   |

In summary, optimum practices of the invention involve a short time solution anneal of the alloys disclosed at about 1850° F. followed by precipitation hardening by heating to about 1300° F. (1275–1350° F.) for about 10 hours.

When thus treated, the high-carbon precipitation-hardening austenitic steels of this invention are characterized by maintenance of high strength for more than 1000 hours at temperatures above 1200° F. and up to about 1500° F., a significant improvement over the presently available steels used for high temperature service.

While I have shown and described several specific embodiments of my invention, it will be understood that these embodiments are merely for the purpose of illustration and description and that various other forms may be devised within the scope of my invention, as defined in the appended claims.

I claim:

1. A precipitation-hardening austenitic iron alloy consisting essentially of, by weight percent

|            |              |
|------------|--------------|
| Carbon     | 0.51 to 0.60 |
| Chromium   | 10.0 to 20.0 |
| Nickel     | 15.0 to 25.0 |
| Zirconium  | 2.0 to 4.0   |
| Titanium   | 2.0 to 4.0   |
| Molybdenum | 2.0 to 4.0   |
| Tungsten   | 2.0 to 4.0   |
| Cobalt     | 2.0 to 4.0   |

with the balance iron and incidental residuals.

2. A precipitation-hardening austenitic iron alloy consisting essentially of, by weight percent

|            |              |
|------------|--------------|
| Carbon     | 0.51 to 0.60 |
| Chromium   | 10.0 to 20.0 |
| Nickel     | 15.0 to 25.0 |
| Zirconium  | 2.0 to 4.0   |
| Titanium   | 2.0 to 4.0   |
| Molybdenum | 2.0 to 4.0   |
| Tungsten   | 2.0 to 4.0   |
| Cobalt     | 2.0 to 4.0   |
| Boron      | Up to .008   |

10 with the balance iron and incidental residuals.

3. A precipitation-hardened austenitic iron alloy consisting essentially of, by weight percent

|            |              |
|------------|--------------|
| Carbon     | 0.51 to 0.60 |
| Chromium   | 10.0 to 20.0 |
| Nickel     | 15.0 to 25.0 |
| Zirconium  | 2.0 to 4.0   |
| Titanium   | 2.0 to 4.0   |
| Molybdenum | 2.0 to 4.0   |
| Tungsten   | 2.0 to 4.0   |
| Cobalt     | 2.0 to 4.0   |

with the balance iron and incidental residuals.

4. A precipitation-hardened austenitic iron alloy consisting essentially of, by weight percent

|            |              |
|------------|--------------|
| Carbon     | 0.51 to 0.60 |
| Chromium   | 10.0 to 20.0 |
| Nickel     | 15.0 to 25.0 |
| Zirconium  | 2.0 to 4.0   |
| Titanium   | 2.0 to 4.0   |
| Molybdenum | 2.0 to 4.0   |
| Tungsten   | 2.0 to 4.0   |
| Cobalt     | 2.0 to 4.0   |
| Boron      | Up to .008   |

with the balance iron and incidental residuals.

#### References Cited by the Examiner

#### UNITED STATES PATENTS

|           |         |              |        |
|-----------|---------|--------------|--------|
| 2,157,060 | 5/1939  | Schafmeister | 75—128 |
| 2,323,490 | 4/1945  | Mohling      | 75—128 |
| 2,617,725 | 11/1952 | Owens        | 75—128 |
| 2,677,610 | 5/1954  | Evans        | 75—128 |

DAVID L. RECK, Primary Examiner.

P. WEINSTEIN, Assistant Examiner.